

## UNITED STATES PATENT OFFICE

2,248,848

## MINERAL OIL COMPOSITION

Ronald Bulkley, Pitman, Lyle A. Hamilton, Wenonah, and Vladimir A. Kalichevsky, Woodbury, N. J., assignors to Socony-Vacuum Oil Company, Incorporated, New York, N. Y., a corporation of New York

No Drawing. Application January 24, 1939,  
Serial No. 252,542

2 Claims. (Cl. 252—46)

This invention is directed to the stabilization of hydrocarbon oils of higher boiling point, such as lubricating oil fractions, against the deteriorating effects of oxidation. Refined oils of the type of turbine oils and the like must be able to withstand the conditions under which they are used without formation of acidic products of a nature corrosive or otherwise damaging to the metal structures to be lubricated by those oils. Moderately refined oils of the nature of many common lubricating fractions must be able to withstand the conditions of their use without the development of similar acidic products. Such acidic products apparently arise from an oxygenation of the oil under its condition of use. This invention is directed to the stabilization against deterioration due to oxidation reactions of any petroleum fractions of a light lubricant nature or heavier, including the variously moderately refined oils, and also inclusive of more highly refined oils such as turbine oils and the like.

This invention has for an important object the preparation of oils falling within the above classes which are stable against oxidation or capable of meeting normal conditions of their use without the formation of materials of an acidic or corrosive nature.

It is known that recent changes in automotive engine design are tending toward higher bearing pressures, higher rotative speeds, higher engine temperatures, and are accompanied by the use of bearing metals less resistant to corrosive materials than those normally used under conditions which are not so prone to develop corrosive oxidation products in the oils. It is also known that an increasing proportion of lubricant oils for all purposes are manufactured by processes of solvent refining or solvent extraction, wherein certain liquid reagents are used to concentrate in the desired lubricant those compounds of a "paraffinic" nature and to reject therefrom the compounds of "naphthenic" nature. These refining processes enable supply of an oil of quite desirable characteristics definitely far superior in general to oils previously produced. It is known that such solvent refined oils are for some reason definitely more prone to the formation of acidic oxidation reaction products of a corrosive nature to bearing metals under conditions of use. This invention is directed to the inhibition of the formation of such acidic reaction products.

We have found that hydrocarbon oils of the

classes defined above, can be stabilized against the formation of acidic reaction products under conditions of use by the addition thereto of relatively minor amounts of oil-soluble sulfonic acids.

The sulfonic acids contemplated are those products which are formed when treating a petroleum lubricant fraction with relatively strong sulfuric acid, such as for example with oleum. In the course of such treatment, as is well known, there are formed sludges and sulfonic acids of various kinds. The sludges, together with the unconsumed acid, are separated from the oil by gravity. This sludge mixture contains certain sulfonic acids which are predominantly of the kind defined as "green sulfonic acids." These green sulfonic acids tend to be more water-soluble than oil-soluble. In the oil which remains after the sludge is withdrawn, there are dissolved other sulfonic acids oil-soluble in nature and generally referred to by the collective terms "brown" or "mahogany sulfonic acids." These oil-soluble sulfonic acids may be recovered by separating them from the oil with an alcohol or with an aqueous alcoholic solution or by neutralizing with an alkali after which the alkaline soaps of sulfonic acids are separated by means of alcohol or aqueous alcoholic solutions and may subsequently be recovered from the solution of acids or solutions of soaps by known processes of acidification, salting out, and dehydration. This invention is directed to the use as stabilizers against the formation of acidic products of minor amounts of such oil-soluble sulfonic acids.

One of the particular tests used for determining the ability of an oil to resist the formation of acidic constituents, is the determination of the neutralization number of the oil after subjecting it to conditions appropriate for its degradation. The neutralization number is defined as the milligrams of potassium hydroxide required to neutralize the acids formed in one gram of oil. As an indication of the efficiency of these inhibitors, there may be cited the following examples:

*Example I*

An oil of the type used in transformers had been highly refined by means of sulfuric acid to a specific gravity of .871, a flash point of 310° F. and a Saybolt viscosity of 69 seconds at 100° F. It was tested by heating 150 grams to 120° C., and bubbling oxygen through it for 70 hours. The degree of oxidation of the oil was measured by

determining the neutralization number of the oxidized oil.

|                          | N. N. |
|--------------------------|-------|
| Oil alone                | 23.0  |
| Oil+.10% sulfonic acids  | 0.03  |
| Oil+.001% sulfonic acids | 2.1   |

*Example II*

A second oil of a Saybolt viscosity of 159 second at 100° F. and a flash point of 410° F. had been moderately refined by means of a solvent. It was tested by heating to 110° C. for three days in the presence of a piece of copper foil and then determining the neutralization number of the oil.

|                         | N. N. |
|-------------------------|-------|
| Oil alone               | 0.19  |
| Oil+.10% sulfonic acids | 0.11  |

It will be seen from these examples that the oils so treated possess considerably enhanced resistance to the formation of acidic products of oxidation.

In general, the amount of sulfonic acids to be used for such purposes is quite small and not in excess of about 0.5% by weight. As a preferred

range we may use from 0.001% to 0.10% by weight.

We claim:

1. A lubricating oil composition relatively stable against the formation of acidic products of oxidation comprising a completely refined lubricating oil which is not so stable, and which oil is initially free of any acidic constituents, and in addition thereto a controlled small amount but not in excess of about 0.5% by weight of oil soluble sulphonated acids derived from the treatment of lubricating oil fractions with relatively strong sulphuric acid.

2. A lubricating oil composition relatively stable against the formation of acidic products of oxidation comprising a completely refined lubricating oil which is not so stable, and which oil is initially free of any acidic constituents, and in addition thereto a controlled small amount from 0.001% to 0.10% by weight of oil soluble sulphonated acids derived from the treatment of lubricating oil fractions with relatively strong sulphuric acid.

RONALD BULKLEY.

LYLE A. HAMILTON.

VLADIMIR A. KALICHEVSKY.